

# UNITED STATES PATENT OFFICE.

S GEE LOWE, OF LOS ANGELES, CALIFORNIA, ASSIGNOR OF ONE-HALF TO JOHN W. FELTES, OF LOS ANGELES, CALIFORNIA.

## CORE-OIL.

1,283,237.

Specification of Letters Patent. Patented Oct. 29, 1918.

No Drawing.

Application filed April 4, 1918. Serial No. 226,785.

*To all whom it may concern:*

Be it known that I, S GEE LOWE, a citizen of the United States, residing at Los Angeles, in the county of Los Angeles and 5 State of California, have invented new and useful Improvements in Core-Oil, of which the following is a specification.

This invention relates to a core oil used in forming cores for making castings.

10 Cores are bodies of sand placed in molds to serve as a part thereof. As they must be molded in a core box, removed therefrom, baked and transferred to the mold, it is necessary to provide a binder for the sand, 15 which will hold the latter together making its removal and transfer possible without its form being destroyed.

The binder should be of such a character that it will not cause the sand to stick to the 20 core box, and will not burn while being baked. In addition to this it should not generate gases by reason of the hot casting metal acting upon it in the mold. Heretofore, linseed oil and fish oil have been used 25 for this purpose. These oils, however, are expensive.

It is an object of this invention to provide a core oil, which will act as a binder, prevent sticking of the sand to the core box, 30 will not burn while the core is being baked, will not generate detrimental gases in use in the mold, and which will be inexpensive.

These objects are accomplished by the core oil whose composition is disclosed hereinafter.

In carrying out this invention a mixture of linseed oil, rosin, distillate and kerosene is formed. A batch of the oil is made in the following proportions, and in the following 40 manner.

To 12½ gallons of linseed oil is added 140 pounds of rosin. The rosin may be of any grade. Before adding the rosin, the linseed oil is brought to the boiling point, and 45 the rosin is added gradually, the boiling being continued until all of the rosin is melted. The composition thus obtained, if allowed to cool, would be viscous. To this composition is added 15½ gallons of distillate. The distillate referred to is that which is derived from the distillation of petroleum and is distilled off at a lower temperature than

kerosene, intermediate benzin and kerosene. This product is marketed under the name of distillate. The distillate is used to cut 55 the rosin and cause it to dissolve. To the composition thus obtained is added 6½ gallons of kerosene. The kerosene so changes the composition that it prevents the sand from sticking to the core box. Kerosene 60 alone, however, will not cut the rosin, and distillate alone will not prevent the sand sticking to core boxes. For this reason both distillate and kerosene are necessary to produce the finished product with all of the desired 65 characteristics.

The rosin used is equivalent in volume to about 17½ gallons. The proportions of ingredients are, therefore: linseed oil 24.05 per centum, rosin 33.65 per centum, distillate 70 29.80 per centum, and kerosene 12.50 per centum by volume.

However, the proportion of linseed oil may be varied. The less the proportion of linseed oil used the greater will be the tendency to burn in baking. The greater the proportion of linseed oil the greater will be the expense.

Instead of linseed oil, other viscous oils may be used, for illustration, paraffin oil. 80 The linseed oil serves the purpose of a slow drier preventing the composition from burning due to fast drying. Any slow drying oil which will dissolve the rosin with the other ingredients mentioned will serve the 85 purpose. I have, therefore, used the term slow drier in the claims to designate this oil.

The proportion of rosin, distillate and kerosene to each other is: rosin 44.30 per centum, distillate 39.24 per centum, and 90 kerosene 16.46 per centum by volume. The proportion of slow drier may be varied depending upon the particular oil used.

What I claim is:

1. A core oil comprising rosin dissolved in 95 a slow drier, distillate and kerosene, said rosin, distillate, and kerosene being in the proportions of substantially 44.30 per centum of rosin, 39.24 per centum of distillate and 16.46 per centum of kerosene by volume. 100

2. A core oil comprising rosin dissolved in linseed oil, distillate, and kerosene being in the proportions of substantially 44.30 per centum of rosin 39.24 per centum of distil-

late and 16.46 per centum of kerosene by volume.

3. A core oil comprising rosin dissolved in linseed oil, distillate, and kerosene, said ingredients being substantially in the proportion of linseed oil 24.05 per centum, rosin 33.65 per centum, distillate 29.80 per cen-

tum, and kerosene 12.50 per centum by volume.

In witness that I claim the foregoing I 10 have hereunto subscribed my name this 25th day of March, 1918.

S GEE LOWE.